



# United States Patent Office.

ADOLPHE JEAN JAMES D'ANDIRAN, OF MULHOUSE, FRANCE.

Letters Patent No. 85,912, dated January 19, 1869.

## IMPROVED MODE OF DYEING COTTON, &c.

The Schedule referred to in these Letters Patent and making part of the same.

To all whom it may concern:

Be it known that I, ADOLPHE JEAN JAMES D'ANDIRAN, have invented "Improvements in the Mode of Dyeing Cotton and other Vegetable Textile Materials," and I do hereby declare that the following is a full and exact description thereof.

I have discovered that artificial colors in general, and more especially those derived from coal, such as aniline violets, blues, and reds, possess the property of combining with madder-mordants on vegetable fibres or tissues previously dyed with madder or its derivatives.

Although the quantities of the artificial coloring-matters which can thus be absorbed are comparatively small, they suffice to modify the original tints, and to produce finer and faster colors than can be economically obtained by any other process.

In mixing the artificial color in solution with the madder or its derivatives, and then dyeing by a single operation, a certain loss of the dye-stuff is sustained. Therefore (without excluding this mode of operating) I prefer, first, to dye the material with madder or its derivatives, and then, after scouring, (and even, if necessary, treating with chloride of lime in the usual manner,) to re-dye it in a fresh bath containing the artificial color.

A simple example will suffice to illustrate the *modus operandi* in all possible applications of my invention.

Supposing, for instance, that it be desired to produce economically a violet shade, as a substitute for that usually obtained with commercial alizarine of the best quality, I begin by weakening the mordants by, say, twenty per cent., thus realizing a first saving of tintorial matter, the oxidation, dunging, or other preliminary treatment of the mordants being effected in the usual manner.

Instead of dyeing with alizarine, I dye with garancine, to which chalk may be added, in case of need, and instead of eight parts of alizarine, which would otherwise have been required, I employ only about five parts of garancine, thus realizing a further saving of three-eighths in weight of dye-stuff.

This fresh saving, added to the previous one, gives a total economy of one-half in weight; that is to say, that instead of two parts of alizarine, I only use one part of garancine, which, as is well known, is a much cheaper product.

The garancine-treatment being completed, the textile material is thoroughly washed, (preferably on the wheel,) and is ready for the second dyeing-process.

To this end, I place in a vat, used solely for this purpose, a sufficient quantity of cold water, and of a solution of from two to three parts of Hoffmann's soluble violet for each thousand parts of the garancine employed in the preceding operation.

If so desired, this violet may be replaced by Perkin's violet, or by rosolane, but in larger proportions; or, again, by soluble Lyons blue, or any other equivalent product.

The textile materials, already dyed with the garancine, as above, are placed in the vat, the contents of which, after having been left cold for some time, to induce a more equal distribution of the violet through the fibres, are rapidly carried to the boiling-point. The ebullition is kept up for from about ten to thirty minutes, according to circumstances, and the dyed goods being then withdrawn, are washed, and treated with chloride of lime in the usual way.

The second dyeing, thus performed, also exercises a cleansing-action, and produces the same effect as the boiling-rinse to which alizarine-violet goods are usually submitted.

The materials then undergo a soap-scouring in cold or tepid water, as a means of increasing the purity of the tones, and of facilitating the subsequent chloride-of-lime treatment, which may, however, be dispensed with when the pattern is free from white.

Having now described and ascertained the nature of my said improvements, and the manner in which they may be carried into effect, I would have it understood that I do not confine myself to the precise details herein laid down, as these may obviously be modified without deviating from the principle of my invention; but

What I claim, and desire to protect by Letters Patent, is—

The application of artificial colors in general, and more especially those derived from coal, (such as aniline violets, blues, and reds,) in combination with madder-mordants, on cotton and other vegetable textile materials previously dyed with madder or its derivatives, substantially in manner and for the purposes herein specified.

ADOLPHE J. J. D'ANDIRAN.

Witnesses:

M. F. MENNONS, Patent Solicitor, Paris.  
T. BESANCON, Clerk to the above.